

111

## UNITED STATES PATENT OFFICE

2,040,795

## TREATMENT OF COTTON GOODS

William Beach Pratt, Wellesley, Mass., assignor  
to John Abbott, Everett D. Chadwick, and  
Marcus B. May, trustees, all of Winchester,  
Mass.

No Drawing. Application July 15, 1932,  
Serial No. 622,831

3 Claims.

(Cl. 8—2)

*404*  
The subject of this invention is the treatment of unbleached cotton goods with a view toward developing such desirable characteristics as cleanliness, softness, absorbency, whiteness and luster therein, while preserving strength, age resistance, and other important physical characteristics. In speaking of "cotton goods," I mean not only piece goods or fabrics, but also yarns such as are intended to enter into fabric-making.

10 In preparing unbleached cotton goods for the market and/or dyeing or other finishing operations, it is customary practice to remove coloring matter and other impurities, including shives and motes, therefrom. Piece goods usually contain sizing agents, such as starch and/or glue, in addition to the original gums and waxes naturally occurring in the cotton fibers, which must be eliminated in order to realize the desired softness and other optimum characteristics in the finished goods. It has been generally the practice to boil cotton goods in caustic soda solutions and then to bleach the washed goods before dyeing and/or marketing them. The boiling treatment in caustic soda solutions must in many cases be performed for a long period of time, not only because it is difficult to wet cotton goods thoroughly, but because some impurities, such as starch sizing, are resistant to removal even by prolonged boiling. The waxes, gums, and resins naturally occurring in cotton fiber also seriously interfere with the wetting of raw cotton goods, as attested by the fact that raw, unsized cotton skeins or piece goods, when put into water or caustic soda solutions, will float for a considerable period of time before they imbibe sufficient water to exercise a tendency to sink. These conditions prevail especially in commercial scale operations involving the boiling treatment of thousands of pounds of cotton goods as a single batch in a kier wherein there is little opportunity for agitation of the caustic soda solution and/or the goods.

I have discovered that in preparing cotton goods of the character described, for subsequent bleaching, more especially with liquors containing oxidizing bleaching agents such as sodium and/or hydrogen peroxide, calcium hypochlorite, chlorine, or the like, it is distinctly advantageous to subject the goods to the action of aqueous solutions of aldehydes. Aside from the fact that such solutions possess the ability to wet the dry goods quickly throughout, especially at elevated temperatures, some of them appear to be selectively absorbed by the cotton fiber so that they cannot be removed by ordinary washing. Fur-

ral, for example, appears to exhibit the property of being selectively absorbed by the cotton fiber from aqueous solution. When the goods, wet with aldehyde, are then subjected to the action of a liquor containing an oxidizing bleach, it is possible to realize goods of excellent whiteness, cleanliness, softness, strength, absorbency, and other desirable physical characteristics. Not only do the shives and motes quickly disappear from the goods in the bleach liquor, but starches and other sizing agents are so completely destroyed that tests show no vestige thereof. It is apparently the case that the aldehyde associated with the goods is transformed by oxidation in situ in the goods into an organic acid, which not only assists the bleaching action, but does so without physical or chemical degradation of the cotton fiber. Then, too, the reaction on the aldehyde taking place quickly in situ in the goods evidently tends to throw off mechanically from the fibers or yarns the shives, motes, sizing or other contaminative matter carried superficially thereon. In the case of starch sizing, it may be that the acid condition developed tends to hydrolyze and dissolve the starch. Whatever may be the chemical and/or physical explanation for the results which I secure, it is a fact that by practicing the steps hereinbefore described, it is possible to secure these results consistently and with various kinds of cotton goods in a period of time which is but a fraction of that required by the usual treatment with caustic followed by bleaching. I have observed that goods processed as hereinbefore described invariably reach a distinctly acid condition at the end of the bleaching operation, despite the fact that the bleach liquor employed, or the goods themselves, may be distinctly alkaline at the beginning of the bleaching operation. This acid condition is attributable to the oxidation of the aldehyde to organic acid in situ in the goods, as hereinbefore described.

The principles of my invention may be applied in various ways and through the use of various aldehydes, but I prefer to work with formaldehyde as my aldehydic agent, primarily because of its low cost as compared with other commercial aldehydes, such as furfural. Unfortunately, however, formaldehyde is an acrid gas and, when used in aqueous solution (formalin), is expelled from the solution rapidly under only moderate heating. Again, formaldehyde is not selectively absorbed by cotton and being miscible with water leaches from the cotton when the latter is placed in a bleach solution. I have discovered, however, that

it is possible to work in a highly practical and satisfactory way with aqueous formaldehyde solutions if they are properly treated with alkalies such as caustic soda or caustic potash. Thus, I 5 have found that by mixing caustic soda or caustic potash and formaldehyde in substantially molecular proportions, together with water in amount to yield an aqueous solution of the desired strength in alkali, and then boiling the mixture, 10 the formaldehyde is quickly converted into a non-volatile reaction product of a dark brown color, which not only behaves like an aldehyde on cotton goods, but is selectively absorbed by the cotton. In commercial practice, it is preferable to use solutions 15 of alkali of about 2% strength, in which case the liquor containing the reaction product may be prepared by using 2 parts by weight of caustic soda to 5 parts by volume of the 40% commercial formaldehyde (formalin) and 100 parts 20 by weight of water. I prefer to use formaldehyde in amount somewhat in excess of the mol. equivalent of the alkali, as this ensures the desired reaction product. It is only for purposes of economy in the aldehyde that it is undesirable and, 25 in fact, unnecessary to use much excess of aldehyde, although the desired reaction seems to go more nearly to completion when as high as two mols of aldehyde are used to one mol. of alkali. On the other hand, I have been unable to realize 30 the desired reaction by having the alkali present in mol. proportion in excess of the formaldehyde. It is quite likely that the caustic soda, under the conditions described, serves to catalyze a condensation or polymerization of the formaldehyde into 35 one or more aldehydes of much higher boiling point, but the condensation reaction seems to go to a definite end point at which the condensation product is soluble in water and imparts a definite depth of coloration thereto. In other words, pro- 40 longed heating of the solution evidently does not conduce to further reaction; and, if the water is evaporated from the solution, it is possible to replace the evaporated water so as to restore the solution to its original dilution. It may be that, 45 in view of the necessity for using mol. equivalents of alkali and formaldehyde, the alkali enters into chemical combination with the formaldehyde, but even if this is the case, the reaction product displays the reacting tendencies of formaldehyde and 50 upon oxidation tends to go to formic acid.

After having produced my dark brown solution containing what may, for convenience, be termed formaldehyde condensation product, I immerse cotton goods in the solution and heat them until 55 they have been thoroughly wetted with the solution throughout. A boiling temperature under atmospheric pressure apparently is sufficient for this purpose. The treated goods may then be drained or squeezed free of excess solution, which 60 can be recovered and reused in the treatment of other cotton goods. The goods wetted with the solution are then put into a suitable oxidizing bleach liquor, such as heretofore used, e. g., containing sodium and/or hydrogen peroxides, calcium hypochlorite, chlorine, or the like. The 65 bleaching operation may be conducted under any suitable conditions of temperature and bleach liquor concentration for a period of time consonant with the attainment of the desired whiteness and brilliancy in the goods. After bleaching, the 70 goods may be washed as ordinarily and, if need be, "soured," to reduce and destroy residual bleach, whereupon they may again be washed and finally dried. As already indicated, the goods take on an acid condition toward the end stages of bleach-

ing, even though they are alkaline as introduced into the bleach liquor, which itself may be initially alkaline. This acid condition is not, however, detrimental to, but, as already stated, enhances characteristics desired in the goods, probably by virtue of the fact that the formic or other organic acid into which the formaldehyde condensation product is oxidized does little, if any, chemical damage to the cotton fiber while increasing its luster or brilliancy, and is substantially completely removed by the washing performed after bleaching. 10

It is possible to practise my invention by adding the cotton goods to a formaldehyde solution before it has undergone the desired reaction, and then to add alkali in appropriate amount and heat the solution so as to bring out the reaction in the presence of the cotton goods. Or the steps may be reversed, with the cotton goods being introduced first into the caustic soda solution, the 15 aldehyde then being added, and heat applied so as to cause the desired reaction.

There are other possible ways of reducing the volatility of formaldehyde solutions so that they can be used more expediently in treating cotton 25 goods. Thus, the addition of soap or other water-soluble colloids to the formaldehyde solution inhibits the liberation of the formaldehyde under heat, but it is distinctly preferable to convert the formaldehyde to the condition resulting from its 30 reaction in the presence of alkali, as hereinbefore described.

While I have mentioned more particularly the availability of formaldehyde, nevertheless one may utilize the higher aldehydes, such for example as acetaldehydes, furfural or butyl aldehyde in the preliminary solution employed before the oxidizing bleach. When an organic acid, such as formic acid, in solution is used as the preliminary treating bath in large scale operations, there is such constant danger of "tendering" the cotton goods that it does not readily lend itself to factory application. But, on the other hand, when such conditions are realized that the cotton after treatment with an aldehyde solution, retains sufficient of the aldehyde for conversion to the acid, there is practically no danger of "tendering" the goods regardless of the time element of the treatment either in the first or second steps of the process. 50

In practising the present invention on a commercial scale, it has been established that the time required for the treatment of cotton goods preliminary to the bleaching operation is only a fraction of that required by a treatment carried out in a comparable way with plain caustic soda solution. That is to say, with a given commercial equipment, for instance a kier designed to hold a number of thousands of pounds of cotton goods and liquor and to be run under particular temperature conditions, circulation of liquor, etc., it is possible to shorten considerably the time period through the use of the preliminary treating liquor of the present invention, and yet to realize a notable improvement in the goods. 55 The present invention thus makes possible not only goods of improved quality, but a reduction in operating costs by virtue of the fact that the capacity of a given equipment is increased. The ratio of liquor to cotton goods is, of course, subject to considerable variation, depending upon the nature of the goods and the kind of equipment employed. In any event, however it is desirable that sufficient liquor be employed to cover or completely submerge the goods so that they 70 75

SEARCH ROOM  
6. BLEACHING & DYEING, FLUID  
TREATMENT & CHEMICAL MODIFI- Cross Reference  
CATION OF TEXTILES & FIBERS,

2,040,795

3

111

will undergo substantially uniform treatment throughout.

The cotton goods processed in accordance with my invention may be straight cotton goods, i. e., 5 piece goods or fabrics containing yarns of only cotton fiber or mixed cotton-rayon goods, i. e., piece goods or fabrics containing besides cotton yarns a proportion of rayon yarns. In the case of the mixed cotton-rayon goods, the rayon as 10 well as the cotton is appreciated in some of the respects hereinbefore noted, although, of course, the rayon does not carry many of the impurities, such as waxes, gums, shives and motes, inherent in raw cotton.

15 What I claim is:

1. A method which comprises polymerizing formaldehyde in aqueous solution into a non-volatile, water-soluble reaction product exhibiting an aldehydic reaction, wetting cotton goods 20 with the resulting solution, and then subjecting

the goods so wetted to the action of oxidizing bleach liquor.

2. A method which comprises treating an aqueous solution of formaldehyde with alkali under conditions to transform the formaldehyde into 5 a non-volatile, water-soluble, colored reaction product, wetting cotton goods with the resulting solution in heated condition, and then subjecting the goods wetted with the solution to the action of an oxidizing bleach liquor.

10 3. A method which comprises heating a mixed solution of formaldehyde and alkali containing substantially mol. proportions of both these agents and of about 2% alkali concentration to convert the formaldehyde into a non-volatile, water-soluble, colored reaction product, wetting cotton goods 15 with the resulting solution in heated condition, and subjecting the goods wetted with the solution to the action of oxidizing bleach liquor.

WILLIAM BEACH PRATT. 20